# EUROPEAN PATENT SPECIFICATION

(11) **EP 2 171 116 B1**
(45) Date of publication and mention of the grant of the patent: **24.08.2011**
(21) Application number: 08762800.4
(22) Date of filing: 06.06.2008
(51) Int. Cl.: C23C 2/02, C23C 2/06, C23C 2/28

(54) **PROCESS FOR MANUFACTURING A GALVANNEALED STEEL SHEET BY DFF REGULATION**
VERFAHREN ZUR HERSTELLUNG EINES VERZINKTEN UND DANN WÄRMEBEHANDELTEN STAHLBLECHS DURCH DFF-REGULIERUNG
PROCÉDÉ DE FABRICATION D'UNE TÔLE D'ACIER RECUITE PAR GALVANISATION PAR RÉGULATION DFF

(30) Priority: 29.06.2007 EP 07290816
(43) Date of publication of application: 07.04.2010
(73) Proprietor: ArcelorMittal France, 93200 Saint Denis (FR); Nippon Steel Corporation, Tokyo 100-8071 (JP)
(72) Inventor: MATAIGNE, Jean-Michel, F-60300 Senlis (FR); BERTRAND, Florence, F-57160 Scy-Chazelles (FR)
(74) Representative: Plaisant, Sophie Marie
(86) International application number: PCT/IB2008/001462
(87) International publication number: WO 2009/004425

(56) References cited:
- EP-A- 0 448 351
- EP-A- 1 612 288
- WO-A-2006/061151
- WO-A-2007/064172
- BE-A3- 1 014 997
- US-A- 3 925 579
- US-A- 3 936 543
- US-A1- 2003 047 255

## Description

The present invention relates to a process for manufacturing a hot-dip galvannealed steel sheet having a TRIP microstructure.

To meet the requirement of lightening power-driven ground vehicle structures, it is known to use TRIP steels (the term TRIP standing for transformation-induced plasticity), which combine very high mechanical strength with the possibility of very high levels of deformation. TRIP steels have a microstructure comprising ferrite, residual austenite and optionally martensite and/or bainite, which allows them to achieve tensile strength from 600 to 1000 MPa. This type of steel is widely used for production of energy-absorbing parts, such as for example structural and safety parts such as longitudinal members and reinforcements.

Before the delivery to car-makers, steel sheets are coated with a zinc-based coating generally performed by hot-dip galvanizing, in order to increase the resistance to corrosion. After leaving the zinc bath, galvanized steel sheets are often submitted to an annealing which promotes the alloying of the zinc coating with the iron of the steel (so-called galvannealing). This kind of coating made of a zinc-iron alloy offers a better weldability than a zinc coating. A Process for manufacturing a hot-dip galvannealed steel sheet is disclosed in BE 1014997 A3.

Most of TRIP steel sheets are obtained by adding a large amount of silicon to steel. Silicon stabilizes the ferrite and the austenite at room temperature, and prevents residual austenite from decomposing to form carbide. However, TRIP steel sheets containing more than 0.2% by weight of silicon, are galvanized with difficulty, because silicon oxides are formed on the surface of the steel sheet during the annealing taking place just before the coating. These silicon oxides show a poor wettability toward the molten zinc, and deteriorate the plating performance of the steel sheet.

To solve this problem, it is known to use TRIP steel having low silicon content (less than 0.2% by weight). However, this has a major drawback: a high level of tensile strength, that is to say about 800 MPa, can be achieved only if the content of carbon is increased. But, this has the effect to lower the mechanical resistance of the welded points.

On the other hand, alloying speed during the galvannealing process is strongly slowed down whatever the TRIP steel composition because of external selective oxidation acting as a diffusion barrier to iron, and the temperature of the galvannealing has to be increased. The increase of the temperature of the galvannealing is detrimental to the preservation of the TRIP effect because of the decomposition of the residual austenite at high temperature. In order to preserve the TRIP effect, a large quantity of molybdenum (more than 0.15 % by weight) has to be added to the steel, so that the precipitation of carbide can be delayed. However, this has an effect on the cost of the steel sheet.

Indeed, the TRIP effect is observed when the TRIP steel sheet is being deformed, as the residual austenite is transformed into martensite under the effect of the deformation, and the strength of the TRIP steel sheet increases.

The purpose of the present invention is therefore to remedy the aforementioned drawbacks and to propose a process for hot-dip galvannealing a steel sheet having a high silicon content (more than 0.5% by weight) and a TRIP microstructure showing high mechanical characteristics, that guarantees a good wettability of the surface steel sheet and no non-coated portions, and thus guarantees a good adhesion and a nice surface appearance of the zinc alloy coating on the steel sheet, and that preserves the TRIP effect.

The first subject of the invention is a process for manufacturing a hot-dip galvannealed steel sheet having a TRIP microstructure comprising ferrite, residual austenite and optionally martensite and/or bainite, said process comprising the steps consisting in:
- providing a steel sheet whose composition comprises, by weight:
   0.01 ≤ C ≤ 0.22%
   0.50 ≤ Mn ≤ 2.0%
   0.5 < Si ≤ 2.0%
   0.005 ≤ Al ≤ 2.0%
   Mo < 0.01 %
   Cr ≤ 1.0%
   P < 0.02%
   Tri ≤ 0.20%
   V ≤ 0.40%
   Ni ≤ 1 .0%
   Nb ≤ 0.20%,
   the balance of the composition being iron and unavoidable impurities resulting from the smelting,
- oxidizing said steel sheet in order to form a layer of iron oxide on the surface of the steel sheet, and to form an internal oxide of at least one type of oxide selected from the group consisting of Si oxide, Mn oxide, Al oxide, complex oxide comprising Si and Mn, complex oxide comprising Si and Al, complex oxide comprising Al and Mn, and complex oxide comprising Si, Mn and Al is formed,
- reducing said oxidized steel sheet in order to reduce the layer of iron oxide,
- hot-dip galvanising said reduced steel sheet to form a zinc-based coated steel sheet, and
- subjecting said zinc-based coated steel sheet to an alloying treatment to form a galvannealed steel sheet.

In order to obtain the hot-dip galvannealed steel sheet having a TRIP microstructure according to the invention, a steel sheet comprising the following elements is provided:
- Carbon with a content between 0.01 and 0.22% by weight. This element is essential for obtaining good mechanical properties, but it must not be present in too large amount in order not to tear the weldability. To encourage hardenability and to obtain a sufficient yield strength Rₑ, and also to form stabilized residual austenite the carbon content must not be less than 0.01% by weight. A bainitic transformation takes place from an austenitic microstructure formed at high temperature, and ferrite/bainite lamellae are formed. Owing to the very low solubility of carbon in ferrite compared with austenite, the carbon of the austenite is rejected between the lamellae. Owing to silicon and manganese, there is very little precipitation of carbide. Thus, the interlamellar austenite is progressively enriched with carbon without any carbides being precipitated. This enrichment is such that the austenite is stabilized, that is to say the martensitic transformation of this austenite does not take place upon cooling down to room temperature.
- Manganese with a content between 0.50 and 2.0% by weight. Manganese promotes hardenability, making it possible to achieve a high yield strength Rₑ. Manganese promotes the formation of austenite, contributes to reducing the martensitic transformation start temperature Ms and to stabilizing the austenite. However, it is necessary to avoid the steel having too high a manganese content in order to prevent segregation, which may be demonstrated during heat treatment of the steel sheet. Furthermore, an excessive addition of manganese causes the formation of a thick internal manganese oxide layer which causes brittleness, and the adhesion of the zinc based coating will not be sufficient.
- Silicon with a content of more than 0.5% by weight, preferably more than 0.6% by weight, and less or equal to 2.0% by weight. Silicon improves the yield strength Rₑ of the steel. This element stabilizes the ferrite and the residual austenite at room temperature. Silicon inhibits the precipitation of cementite upon cooling from austenite, considerably retarding the growth of carbides. This stems from the fact that the solubility of silicon in cementite is very low and the fact that silicon increases the activity of the carbon in austenite. Thus, any cementite nucleus that forms will be surrounded by a silicon-rich austenitic region, and rejected to the precipitate-matrix interface. This silicon-enriched austenite is also richer in carbon, and the growth of the cementite is slowed down because of the reduced diffusion resulting from the reduced carbon activity gradient between the cementite and the neighbouring austenitic region. This addition of silicon therefore contributes to stabilizing an amount of residual austenite sufficient to obtain a TRIP effect. During the annealing step to improve the wettability of the steel sheet, internal silicon oxides and complex oxide comprising silicon and/or manganese and/or aluminium are formed and dispersed under the surface of the sheet. However, an excessive addition of silicon causes the formation of a thick internal silicon oxide layer and possibly complex oxide comprising silicon and/or manganese and/or aluminium which causes brittleness and the adhesion of the zinc based coating will not be sufficient.
- Aluminium with a content between 0.005 and 2.0% by weight. Like the silicon, aluminium stabilizes ferrite and increases the formation of ferrite as the steel sheet cools down. It is not very soluble in cementite and can be used in this regard to avoid the precipitation of cementite when holding the steel at a bainitic transformation temperature and to stabilize the residual austenite. A minimum amount of aluminium is required in order to deoxidize the steel.
- Molybdenum with a content less than 0.01 % by weight, and preferably not exceeding 0.006% by weight. Conventional process requires the addition of Mo to prevent carbide precipitation during re-heating after galvanizing. Here, thanks to the internal oxidation of silicon, manganese and aluminium, the alloying treatment of the galvanized steel sheet can be performed at a lower temperature than that of conventional galvanized steel sheet comprising no internal oxide. Consequently, the content of molybdenum can be reduced and be less than 0.01% by weight, because it is not necessary to delay the bainitic transformation as it is the case during the alloying treatment of conventional galvanized steel sheet.
- Chromium with a content not exceeding 1.0% by weight. The chromium content must be limited in order to avoid surface appearance problems when galvanizing the steel
- Phosphorus with a content not exceeding 0.02% by weight, and preferably less than 0.010% by weight. Phosphorus in combination with silicon increases the stability of the residual austenite by suppressing the precipitation of carbides.
- Titanium with a content not exceeding 0.20% by weight. Titanium improves the yield strength of Rₑ, however its content must be limited to 0.20% by weight in order to avoid degrading the toughness.
- Vanadium with a content not exceeding 0.40% by weight. Vanadium improves the yield strength of Rₑ by grain refinement, and improves the weldability of the steel. However, above 0.40% by weight, the toughness of the steel is degraded and there is a risk of cracks appearing in the weld zones.
- Nickel with a content not exceeding 1.0% by weight. Nickel increases the yield strength of Rₑ. Its content is generally limited to 1.0% by weight because of its high cost.
- Niobium with a content not exceeding 0.20% by weight. Niobium promotes the precipitation of carbonitrides, thereby increasing the yield strength of Rₑ. However, above 0.20% by weight, the weldability and the hot formability are degraded.

The balance of the composition consists of iron and other elements that are usually expected to be found and impurities resulting from the smelting of the steel, in proportions that have no influence on the desired properties.

The steel sheet having the above composition is first subjected to an oxidation followed by a reduction, before being hot-dip galvanized in a bath of molten zinc and heat-treated to form said galvannealed steel sheet.

The aim is to form an oxidized steel sheet having an outer layer of iron oxide with a controlled thickness which will protect the steel from the selective outer oxidation of silicon, manganese and aluminium, while the steel sheet is annealed before the hot-dip galvanization.

Said oxidation of the steel sheet is performed under conditions that allow the formation, on the surface of the steel sheet, of a layer of iron oxide containing no superficial oxides selected from the group consisting of silicon oxide, manganese oxide, aluminium oxide, complex oxide comprising silicon and/or manganese and/or aluminium. During this step, internal selective oxidation of silicon, manganese and aluminium will develop under the iron oxide layer, and leads to a deep depletion zone in metallic silicon, manganese and aluminium which will minimize the risk of superficial selective oxidation when the further reduction will be achieved. A layer of an internal oxide of at least one type of oxide selected from the group consisting of silicon oxide, manganese oxide, aluminium oxide, complex oxide comprising Si and Mn, complex oxide comprising Si and Al, complex oxide comprising Mn and Al and complex oxide comprising Si, Mn and Al is thus formed.

The oxidation is preferably performed by heating said steel sheet from ambient temperature to a heating temperature T1 which is between 680 and 800°C, in a direct flame furnace where the atmosphere comprises air and fuel, with a ratio air-to-fuel preferably between 1 and 1.2.

When the temperature T1 is above 800°C, the iron oxide layer formed on the surface of the steel sheet will contain manganese coming from the steel, and the wettability will be impaired. If the temperature T1 is below 680°C, the internal oxidation of silicon, manganese and aluminium will not be favoured, and the galvanizability of the steel sheet will be insufficient.

An atmosphere having a ratio air-to-fuel less than 1 leads to the formation of superficial oxidation of silicon, manganese and aluminium, and thus a superficial layer of oxides selected from the group consisting of silicon oxide, manganese oxide, aluminium oxide, and complex oxide comprising silicon and/or manganese and/or aluminium, possibly in combination with iron oxide is formed, and the wettability is impaired. However, with a ratio air-to-fuel above 1.2, the layer of iron oxide is too thick, and will not be completely reduced. Thus, the wettability will also be impaired.

When leaving the direct flame furnace, the oxidized steel sheet is reduced in conditions permitting the achievement of the complete reduction of the iron oxide into iron. This reduction step can be performed in a radiant tube furnace or in a resistance furnace. Said oxidized steel sheet is thus heat treated in an atmosphere comprising preferably more than 15% by volume of hydrogen, the balance being nitrogen and unavoidable impurities. Indeed, if the content of hydrogen in the atmosphere is less than 15% by volume, the layer of iron oxide can be insufficiently reduced and the wettability is impaired.

Said oxidized steel sheet is heated from the heating temperature T1 to a soaking temperature T2, then it is soaked at said soaking temperature T2 for a soaking time t2, and is finally cooled from said soaking temperature T2 to a cooling temperature T3.

Said soaking temperature T2 is preferably between 770 and 850°C. When the steel sheet is at the temperature T2, a dual phase microstructure composed of ferrite and austenite is formed. When T2 is above 850°C, the volume ratio of austenite grows too much, and external selective oxidation occurs on the steel surface. But when T2 is below 770°C, the time required to form a sufficient volume ratio of austenite is too high.

In order to obtain the desired TRIP effect, sufficient austenite must be formed during the soaking step, so that sufficient residual austenite is maintained during the cooling step. The soaking is performed for a time t2, which is preferably between 20 and 180s. If the time t2 is longer than 180s, the austenite grains coarsen and the yield strength Rₑ of the steel after forming will be limited. Furthermore, the hardenability of the steel is low. However, if the steel sheet is soaked for a time t2 less than 20s, the proportion of austenite formed will be insufficient and sufficient residual austenite and bainite will not form when cooling.

The reduced steel sheet is finally cooled at a cooling temperature T3 near the temperature of the bath of molten zinc, in order to avoid the cooling or the re-heating of said bath. T3 is thus preferably between 460 and 510°C. Therefore, a zinc-based coating having a homogenous microstructure can be obtained.

When the steel sheet is cooled, it is hot dipped in the bath of molten zinc whose temperature is preferably between 450 and 500°C. This bath can contain 0.08 to 0.135% by weight of dissolved aluminium, the balance being zinc and unavoidable impurities. Aluminium is added in the bath in order to deoxidize the molten zinc, and to make it easier to control the thickness of the zinc-based coating. In that condition, precipitation of delta phase (FeZn₇) is induced at the interface of the steel and of the zinc-based coating.

When leaving the bath, the steel sheet is wiped by projection of a gas, in order to adjust the thickness of the zinc-based coating. This thickness, which is generally between 3 and 10 µm, is determined according to the required resistance to corrosion.

The hot-dip galvanized steel sheet is finally heat-treated so that a coating made of a zinc-iron alloy is obtained, by diffusion of the iron from steel to the zinc of the coating. This alloying treatment can be performed by maintaining said steel sheet at a temperature T4 between 460 and 510°C for a soaking time t4 between 10 and 30s. Thanks to the absence of external selective oxidation of silicon, manganese and aluminium, this temperature T4 is lower than the conventional alloying temperatures. For that reason, large quantities of molybdenum to the steel are not required, and the content of molybdenum in the steel can be limited to less than 0.01 % by weight. If the temperature T4 is below 460°C, the alloying of iron and zinc is not possible. If the temperature T4 is above 510°C, it becomes difficult to form stable austenite, because of the unwished carbide precipitation, and the TRIP effect cannot be obtained. The time t4 is adjusted so that the average iron content in the alloy is between 8 and 12% by weight, which is a good compromise for improving the weldability of the coating and limiting the powdering while shaping.

The invention will now be illustrated by examples given by way of nonlimiting indication and with reference to figures 1 and 2.

Trial was carried out using samples A and B coming from 0.8 mm thick sheet manufactured from a steel sheet whose composition is given in table I.

Samples A and B are pre-heated from ambient temperature (20°C) to 750°C, in a direct flame furnace. They are subsequently and continuously annealed in a radiant tube furnace, where they are heated from 750° to 800°C, then they are soaked at 800°C for 60 s, and finally they are cooled to 460 °C. The atmosphere in the radiant tube furnace comprises 30% by volume of hydrogen, the balance being nitrogen and unavoidable impurities.

After cooling, samples A and B are hot dip galvanized in a molten zinc-based bath comprising 0.12% by weight of aluminium, the balance being zinc and unavoidable impurities. The temperature of said bath is 460 °C. After wiping with nitrogen and cooling the zinc-based coating, the thickness of the zinc-based coating is 7 µm.

First, the aim is to compare the wettablilty and the adherence of these samples, when the air-to-fuel ratio in the direct flame furnace fluctuates. The air-to-fuel ratio is 0.90 for sample A, and 1.05 according to the invention for sample B. The results are shown in table II.

The wettability is visually controlled by an operator. The adherence of the coating is also visually controlled after a 180° bending test of samples.

Table I: chemical composition of the steel of samples A and B, in % by weight, the balance of the composition being iron and unavoidable impurities (sample A and B).

**Table I**

| C | Mn | Si | Al | Mo | Cr | P | Ti | V | Ni | Nb |
|---|---|---|---|---|---|---|---|---|---|---|
| 0.20 | 1.73 | 1.73 | 0.01 | 0.005 | 0.02 | 0.01 | 0.005 | 0.005 | 0.01 | 0.005 |

**Table II**

| | **Wettabilty** | **Adherence** | **Aspect of the surface** |
|---|---|---|---|
| **Sample A**** | Bad | Bad | Bad |
| **Sample B*** | Good | Good | Good |

| | | | |
|---|---|---|---|
| * according to the invention ** according to the conventional process | | | |

Figure 1 is a photography of sample A after the pre-heating step and before the annealing step, and figure 2 is a photography of sample B after the pre-heating step and before the annealing step.

Then, the aim is to show the effect of the internal selective oxidation of silicon and manganese on the temperature of alloying. Thus, the temperature of alloying treatment applied to sample B in order to obtain a galvannealed steel sheet according to the invention is compared with the temperature of alloying of sample A.

Sample B which has been hot dip galvanized is then subjected to an alloying treatment by heating it to 480°C, and by maintaining it at this temperature for 19 s . The inventors have checked that the TRIP microstructure of the obtained hot dip galvannealed steel sheet according to the invention was not lost by this alloying treatment.

In order to obtain the alloying of the zinc-based coating of sample A, it is necessary to heat it to 540°C, and to maintain it at this temperature for 20 s With such a treatment, the inventors have checked that carbide precipitation occurs, residual austenite is no more kept during cooling down to room temperature and that the TRIP effect has disappeared.

## Claims

1. Process for manufacturing a hot-dip galvannealed steel sheet having a transformation-induced plasticity (TRIP)microstructure comprising ferrite, residual austenite and optionally martensite and/or bainite, said process comprising the steps consisting in:
- providing a steel sheet whose composition comprises, by weight:
0.01 ≤ C ≤ 0:22%
0.50 ≤ Mn ≤ 2.0%
p.5 ≤ Si ≤ 2.0%
0.005 ≤ Al ≤ 2.0
Mo < 0.01%
Cr ≤ 1.0%
P < 0.02%
Ti ≤ 0.20%
v ≤ 0.40%
Ni ≤ 1.0%
Nb ≤ 0.20%,
the balance of the composition being iron and unavoidable impurities resulting from the smelting,
- oxidizing said steel sheet by heating it from ambient temperature to a temperature T1 between 680 to 800°C, in a direct flame furnace where the atmosphere comprises air and fuel with an air-to-fuel ratio between 1.0 and 1.2 in order to form a layer of iron oxide on the surface of the steel sheet, and to form an internal oxide of at least one type of oxide selected from the group consisting of Si oxide, Mn oxide, Al oxide, complex oxide comprising Si and Mn, complex oxide comprising Si and Al, complex oxide comprising Al and Mn, and complex comprising Si, Mn and Al,
- reducing said oxidized steel sheet in order to reduce the layer of iron oxide,
- hot-dip galvanising said reduced steel sheet to form a zinc-based coated steel sheet, and
- subjecting said zinc-based coated steel sheet to an alloying treatment to form a galvannealed steel sheet.

2. Process according to claim 1, wherein said steel sheet comprises, in % by weight, P < 0.010%.

3. Process according to claim 1 or 2, wherein said steel sheet comprises, in % by weight, Mo≤ 0.006%.

4. Process according to any one of claims 1 to 3, wherein the reduction of said oxidized steel sheet consists of a heat treatment performed in an atmosphere comprising more than 15% by volume of hydrogen, the balance being nitrogen and unavoidable impurities, said heat treatment comprising a heating phase from the temperature T1 to a soaking temperature T2, a soaking phase at said soaking temperature T2 for a soaking time t2, and a cooling phase from said soaking temperature T2 to a cooling temperature T3.

5. Process according to claims 4, wherein said soaking temperature T2 is between 770 and 850°C.

6. Process according to claim. 4 or 5, wherein said soaking time t2 is between 20 and 180 s.

7. Process according to any one of claims 4 to 6, wherein said cooling temperature T3 is between 460 to 510°C.

8. Process according to any one of claims 3 to 7, wherein said reduction is performed in a radiant tube furnace or in a resistance furnace.

9. Process according to any one of claims 1 to 8, wherein the hot-dip galvanizing is performed by hot-dipping said reduced steel sheet in a molten bath comprising 0.08 to 0.135% by weight of aluminium, the balance being zinc and unavoidable impurities.

10. Process according to claim 9, wherein the temperature of said molten bath is between 450 and 500°C.

11. Process according to any one of claims 1 to 10, wherein said alloying treatment is performed by heating said zinc-based coated steel sheet at a temperature T4 between 460 and 510°C for a soaking time t4 between 10 and 30 s.

## Patentansprüche

1. Prozess zum Herstellen eines schmelzgetauchten galvanisch getemperten (galvannealed) Stahlblechs, das eine durch Transformation induzierte Plastizitäts-(TRIP)-Mikrostruktur hat, die Ferrit, Restaustenit und optional Martensit und/oder Balnit umfasst, wobei der Prozess die Schritte umfasst, die aus Folgendem bestehen:
- Bereitstellen eines Stahlblechs, dessen Zusammensetzung Folgendes in Gewichts-% umfasst:
0,01 ≤ C ≤ 0,22%
0,50 ≤ Mn ≤ 2,0%
0,5 < Si ≤ 2,0%
0,005 ≤ A1 ≤ 2,0
Mo < 0,01%
Cr ≤ 1,0%
P < 0,02%
T2 ≤ 0,20%
V ≤ 0,40%
Ni ≤ 1,0%
Nb ≤ 0,20%,
wobei der Rest der Zusammensetzung Eisen und unvermeidliche Verunreinigungen sind, die aus dem Verhütten herrühren,
- Oxidieren des Stahlblechs durch Erwärmen desselben von Umgebungstemperatur auf eine Temperatur T1 zwischen 680 und 800°C im Direktflammenofen, in dem die Atmosphäre Luft und Brennstoff in einem Luft-Brennstoff-Verhältnis zwischen 1,0 und 1,2 umfasst, um eine Schicht von Eisenoxid auf der Oberfläche des Stahlblechs zu bilden und um ein inneres Oxid des mindestens einen Typs von Oxid zu bilden, das aus der Gruppe bestehend Si-Oxid, Mn-Oxid, Al-Oxid, Komplexoxid, das Si und Mn umfasst, Komplexoxid, das Si und Al umfasst, Komplexoxid, das Al und Mn umfasst, und Komplexoxid, das Si, Mn und Al umfasst, ausgewählt ist,
- Reduzieren des oxidierten Stahlblechs, um die Schicht von Eisenoxid zu reduzieren,
- Feuermetallisieren des reduzierten Stahlblechs, um ein zinkbasiertes beschichtetes Stahlblech zu bilden, und
- Einwirkenlassen einer Legierungsbehandlung auf das zinkbasierte beschichtete Stahlblech, um ein galvannealed Stahlblech zu erhalten.

2. Prozess nach Anspruch 1, wobei das Stahlblech P < 0,010% in Gewichts-% umfasst.

3. Prozess nach Anspruch 1 oder 2, wobei das Stahlblech Mo≤ 0,006% in Gewichts-% umfasst.

4. Prozess nach einem der Ansprüche 1 bis 3, wobei das Reduzieren des oxidierten Stahlblechs aus einer Wärmebehandlung besteht, die in einer Atmosphäre ausgeführt wird, welche mehr als 15 Volumen-% Wasserstoff umfasst, wobei der Rest Stickstoff und unvermeidliche Verunreinigungen sind, wobei die Wärmebehandlung eine Heizphase von der Temperatur T1 bis zu einer Haltetemperatur T2, eine Haltephase bei der Haltetemperatur T2 für eine Haltezeit t2 und eine Kühlungsphase von der Haltetemperatur T2 bis zu einer Kühltemperatur T3 umfasst.

5. Prozess nach Anspruch 4, wobei die Haltetemperatur T2 zwischen 770 und 850°C liegt.

6. Prozess nach Anspruch 4 oder 5, wobei die Haltezeit t2 zwischen 20 und 180 s liegt.

7. Prozess nach einem der Ansprüche 4 bis 6, wobei die Kühltemperatur T3 zwischen 460 und 510°C liegt.

8. Prozess nach einem der Ansprüche 3 bis 7, wobei das Reduzieren in einem Strahlrohrofen oder in einem Widerstandsofen ausgeführt wird.

9. Prozess nach einem der Ansprüche 1 bis 8, wobei das Feuermetallisieren durch Schmelztauchen des reduzierten Stahlblechs in ein Schmelzbad ausgeführt wird, das 0,08 bis 0,135 Gewichts-% Aluminium umfasst, wobei der Rest Zink und unvermeidliche Verunreinigungen sind.

10. Prozess nach Anspruch 9, wobei die Temperatur des Schmelzbades zwischen 450 und 500°C liegt.

11. Prozess nach einem der Ansprüche 1 bis 10, wobei die Legierungsbehandlung durch Erwärmen des zinkbasierten beschichteten Stahlblechs auf eine Temperatur T4 zwischen 460 und 510°C für eine Haltezeit t4 zwischen 10 und 30 s ausgeführt wird.

## Revendications

1. Procédé pour fabriquer une tôle d'acier galvanisé-allié ayant une microstructure à plasticité induite par transformation (TRIP) comprenant de la ferrite, de l'austénite résiduelle et éventuellement de la martensite et/ou de la bainite, ledit procédé comprenant les étapes consistant à :
- approvisionner une tôle d'acier dont la composition comprend, en poids :
0,01 ≤ Cl 0,22 %
0,50 ≤ Mn ≤ 2,0 %
0,5 < Si ≤ 2,0 %
0,005 ≤ A1 ≤ 2,0 %
Mo < 0,01 %
Cr ≤ 1,0 %
P < 0,02 %
Ti ≤ 0,20 %
V ≤ 0,40 %
N ≤ 1,0 %
Nb ≤ 0,20 %
le solde de la composition étant du fer et les inévitables impuretés résultant de la fusion,
- oxyder ladite tôle d'acier en la chauffant de la température ambiante à une température T1 comprise entre 680 et 800 °C, dans un four à flamme directe où l'atmosphère comprend de l'air et un combustible avec un rapport air sur combustible compris entre 1,0 et 1,2 afin de former une couche d'oxyde de fer sur la surface de la tôle d'acier, et de former un oxyde interne d'au moins un type d'oxyde choisi dans le groupe constitué par un oxyde de Si, un oxyde de Mn, un oxyde d'Al, un oxyde complexe comprenant Si et Mn, un oxyde complexe comprenant Si et Al, un oxyde complexe comprenant Al et Mn, et un oxyde complexe comprenant Si, Mn et Al,
- réduire ladite tôle d'acier oxydé afin de réduire la couche d'oxyde de fer,
- galvaniser à chaud au trempé ladite tôle d'acier réduit pour former une tôle d'acier avec revêtement à base de zinc, et
- soumettre ladite tôle d'acier avec revêtement à base de zinc à un traitement d'alliation pour former une tôle d'acier galvanisé-allié.

2. Procédé selon la revendication 1, dans lequel ladite tôle d'acier comprend, en % en poids, P < 0,010 %.

3. Procédé selon la revendication 1 ou 2, dans lequel ladite tôle d'acier comprend, en % en poids, Mo ≤ 0,006 %.

4. Procédé selon l'une quelconque des revendications 1 à 3, dans lequel la réduction de ladite tôle d'acier oxydé consiste en un traitement thermique effectué dans une atmosphère comprenant plus de 15 % en volume d'hydrogène, le solde étant de l'azote et les inévitables impuretés, ledit traitement thermique comprenant une phase de chauffage de la température T1 à une température d'égalisation T2, une phase d'égalisation à ladite température d'égalisation T2 pendant un temps d'égalisation t2, et une phase de refroidissement de ladite température d'égalisation T2 à une température de refroidissement T3.

5. Procédé selon la revendication 4, dans lequel ladite température d'égalisation T2 se situe entre 770 et 850 °C.

6. Procédé selon la revendication 4 ou 5, dans lequel ledit temps d'égalisation t2 se situe entre 20 et 180 s.

7. Procédé selon l'une quelconque des revendications 4 à 6, dans lequel ladite température de refroidissement T3 se situe entre 460 et 510 °C.

8. Procédé selon l'une quelconque des revendications 3 à 7, dans lequel ladite réduction est effectuée dans un four à tubes radiants ou dans un four à résistance.

9. Procédé selon l'une quelconque des revendications 1 à 8, dans lequel la galvanisation à chaud est effectuée en trempant ladite tôle d'acier réduit dans un bain fondu comprenant 0,08 à 0,135 % en poids d'aluminium, le solde étant du zinc et les inévitables impuretés.

10. Procédé selon la revendication 9, dans lequel la température dudit bain fondu se situe entre 450 et 500 °C.

11. Procédé selon l'une quelconque des revendications 1 à 10, dans lequel ledit traitement d'alliage est réalisé en chauffant ladite tôle d'acier avec revêtement à base de zinc à une température T4 comprise entre 460 et 510 °C pendant un temps d'égalisation t4 compris entre 10 et 30 s.
